

## UNITED STATES PATENT OFFICE

2,527,141

TREATMENT OF COTTON FABRICS WITH  
UREA-ALKALI-ZINCATE SOLUTION

Charles L. Mantell, Manhasset, and Oscar K. Heim, Woodside, N. Y., assignors to United Merchants & Manufacturers, Inc., Wilmington, Del., a corporation of Delaware

No Drawing. Application May 10, 1949,  
Serial No. 92,511

20 Claims. (Cl. 8—116.2)

1

This invention relates to the treatment of cotton fabrics and has for its primary object a method of modifying the normal characteristics of woven or knitted cotton cloth to the end of producing a fabric of enhanced value and utility, the method requiring no complicated or special equipment for its practice and being otherwise economical to carry out. As hereinafter described in greater detail, the invention contemplates the treatment of the fabric with a solution which, in more or less noticeable degree according to the character of the fabric and the method employed, produces some or all of the effects of modifying the shrinkage characteristics of the fabric, eliminating fuzz, and rendering the fabric stiffer and somewhat translucent.

The invention essentially comprises a process of treating cotton fabric with a solution containing caustic zincate and urea, hereinafter referred to as the treating solution, there being obtained a fabric having, among other effects, appreciably modified shrinkage characteristics; that is, it shows a substantially reduced shrinkage by comparison with the normal shrinkage of the untreated fabric, considering such normal shrinkage to be the initial wash shrinkage. In addition, the treated fabric has a more clearcut and attractive appearance. Thus, when the untreated fabric is held up to the light and examined, i. e., held between the light and the eye, it presents a misty appearance due to the lack of sharp definition of the warp and weft thread outlines which results from the fuzz on the threads. This characteristic is particularly evident when such fabrics are used, for example, as curtains. It has been found, according to this invention, that if the fabric is treated as described, its appearance is quite radically changed. When the fabric so treated is held up to the light and examined as before, it is observed that the threads are sharply outlined, there being substantially no evidence of fuzz. It has also been observed in some instances that, notwithstanding the sharpening of the outlines of the threads, the body of each thread assumes a somewhat translucent character. As will be understood, these last mentioned effects will each be more or less noticeable and of varying practical consequence depending on the character of the fabric and the use to which it is put;

but, for convenience, they may be described as bringing about a clarification of the fabric.

It has further been observed that the treated fabric tends to become stiffer by comparison with the untreated fabric. Stiffness is a desirable characteristic in certain materials, for example in curtain and table goods and in certain types of dresses and blouses, e. g., lawns and organdies.

Besides the above-mentioned solution treating process, the invention also comprises the combination therewith of one or more other steps as modifications of the process. Such modified processes may comprise (1) a preliminary chemical degradation step followed by the solution treating step; and (2) a preliminary chemical degradation step, the solution treating step, and treatment with a special stiffening liquor. While the effects achieved by means of the solution treating process are noteworthy in themselves, it has been found that additional advantages may be realized by means of the modified processes. Each of these processes will be hereinafter described in relation to the treatment of an open weave cotton fabric, but it is to be understood, of course, that the advantages of the invention may be obtained with cotton fabrics in general.

As described, the treating solution is composed of caustic zincate and urea. It may be prepared by mixing together an aqueous solution of urea and an alkali metal zincate selected from the class consisting of sodium zincate and potassium zincate; or by adding zinc oxide to an aqueous solution of an alkali metal hydroxide selected from the class consisting of sodium hydroxide and potassium hydroxide, sodium zincate and potassium zincate respectively being formed, and then incorporating the urea. It is to be understood that in referring to the zinc oxide content of the solution it is intended to include the oxide added as such or as comprised in the alkali metal zincate added to the solution or formed therein. Compounds which, when added to a caustic zincate solution, hydrolyze to form urea, may be used in making up the solvent. Such compounds may include, for example, cyanamide, guanidine, guanylurea, etc. In the premises, it will be understood that the term "urea" as used herein is intended to include urea per se and also compounds which produce urea as in the foregoing manner. The amount of urea may be varied from about

## 3

2 to about 20% by weight. At concentrations below this range, the solution has decreased effects, while at concentrations above 20%, no worthwhile improvements result. Zinc oxide, whether added as such or in the form of the zincate, may be present in amounts ranging from about 2 to about 10% by weight, calculated as zinc oxide; while the caustic may be varied from about 6 to about 28% by weight or more, although the use of higher concentrations of caustic generally does not justify the added expense involved. If sodium hydroxide is employed as the caustic, a preferred concentration is from about 6 to about 20%; for potassium hydroxide a preferred range is from about 8 to about 28%. As in the case of urea, the effects are decreased by going below the minimum concentrations of the latter materials; above the maximum concentrations given, there is no worthwhile improvement in results. A preferred solution is one containing about 10% urea, about 6% zinc oxide, and about 12% caustic.

Application of the solution to the fabric is done by simply pouring it on the fabric, although usually it is better to rub it on, either manually or by means of knives or doctor blades. Mangle equipment such as paddlers or quetches are useful for this purpose, as is also pressure equipment like rollers. Jigs and rolls are likewise suitable. The fabric may or may not be under tension during the application of the solution. Preferably it is not. The time of treatment is not critical and may range from about 1 second up to 24 hours or more, and may conveniently be in the range of 1 second to 1 hour. The treating temperature used is generally room temperature, although, of course, higher and lower temperatures, say from the freezing point to 120° F., may be employed. After treating, the solution may be allowed to dry on the fabric or not, as desired. The goods then may be neutralized, rinsed and dried; or neutralized and dried; or washed and dried. Moreover, in any sequence of these steps and at any stage thereof, the goods in process may or may not be under tension. Thus after the treating solution has been applied, the following alternative procedures or variations may be employed.

1. Dry under tension, neutralize, rinse, dry. 2. Dry under tension, neutralize, dry. 3. Dry under tension, wash, dry. 4. Dry without tension, neutralize, rinse, dry. 5. Dry without tension, neutralize, dry. 6. Dry without tension, wash, dry. 7. Neutralize, rinse, dry. 8. Neutralize, dry. 9. Wash, dry. In further variations of the procedure, as indicated, the neutralizing, rinsing, washing and final drying steps may each be done while the material is in either a stretched or unstretched condition. The preferred method is as follows: Dry under tension, for example on a tenter or drying can, neutralize with dilute acid and rinse with water, the neutralization and rinsing being done while the fabric is in an unstretched condition, and frame dry.

The following example illustrates the improvement with respect to fabric shrinkage obtainable by the invention.

## Example 1

Cotton marquisette containing starch was held under moderate tension on a frame and treated at room temperature with an aqueous solution containing 10% urea, 4.5% zinc oxide and 10% caustic soda. The solution was poured over the cloth for about two minutes and then the cloth was washed with cold water and 1% acetic acid

4  
5 to remove the alkali and zinc. The goods were further washed with cold water until neutral and dried in warm air at about 100° F. Another sample of marquisette was treated the same way after first removing the starch. The results follow:

|                                               | Shrinkage, in percent |         |
|-----------------------------------------------|-----------------------|---------|
|                                               | Warp                  | Filling |
| 10                                            |                       |         |
| Original cloth, containing starch.....        | 15.3                  | 12.7    |
| Treated cloth.....                            | 5.8                   | 4.4     |
| Treated cloth, starch previously removed..... | 3.9                   | 2.3     |

15 The shrinkages reported were obtained according to A. S. T. M. D437-36. By the term "cotton marquisette containing starch" is meant either a fabric in its grey stage from which the starch is used as a sizing on the yarn has not been removed, or a semi-finished fabric to which starch has been applied, or a finished fabric to which the starch has been applied as a finish. In addition, unsized, desized, and unfinished goods may be treated in the manner described.

20 25 If the treating solution is not washed from the cloth but dried on instead, as is presently preferred, a lower shrinkage effect may be realized. The following example illustrates this variation in procedure:

## Example 2

30 35 Cotton marquisette that had been kier-boiled and partially mercerized according to conventional practice was subjected to treatment with the solution employed in Example 1. One sample of cloth was treated with the solution for about one minute at 25° C., and then washed and dried as above described. A second sample was 40 treated with solution for about one minute at 25° C., then warmed at 260° F. until the cloth was just dry, and thereafter washed and dried as the first sample. The first sample showed a warp shrinkage of 10.3% and a filling shrinkage of 7.7%; the second showed a warp shrinkage of 6.6% and a filling shrinkage of 7.4%. Shrinkage was determined according to A. S. T. M. D437-36. The results obtained with the second sample were 45 50 duplicated with a solution of somewhat different composition, namely, 2.6% zinc oxide, 7.4% caustic, and 5% urea, the procedure being otherwise the same. It was further noticed that when the solution was dried on the cloth, better stiffness was obtained.

55 60 In each of the foregoing examples the visual characteristics of the treated cloth are appreciably altered. By comparison with the original material, the treated cloth has a cleaner thread outline and an overall translucent appearance. These effects are produced in addition to the effects of shrinkage control or dimensional stability and stiffness. By modifying the foregoing process it has been found that the latter effects may be favorably increased.

65 Other examples are as follows:

## Example 3

70 75 Samples of a leno weave cotton marquisette, which previously had been mercerized, kier-boiled and bleached according to conventional mill practice, were held under moderate tension on a frame and treated at room temperature with various solutions, the composition of which applied 75 pears below. The solutions were poured over the

stretched fabrics for one minute, the fabrics dried at 240° F., then removed from the stretchers and neutralized with dilute sulfuric acid, rinsed with cold water, reframed and dried at 240° F. A control sample was treated with water instead of solution. Shrinkage, tensile strength (warp) and stiffness data were then obtained on the samples. The results are as follows:

| Solution Composi-<br>tion |     |      | Shrinkage<br>Per Cent |         | Tensile<br>Strength | Stiffness<br>Coeffi-<br>cient |
|---------------------------|-----|------|-----------------------|---------|---------------------|-------------------------------|
| NaOH                      | ZnO | Urea | Warp                  | Filling |                     |                               |
| 6                         | 2   | 2    | 7.2                   | 9.3     | 23.4                | 0.50                          |
| 6                         | 2   | 20   | 6.5                   | 11.0    | 28.8                | 0.65                          |
| 20                        | 10  | 2    | 5.2                   | 10.7    | 27.7                | 1.46                          |
| 20                        | 10  | 20   | 5.5                   | 8.3     | 30.9                | 1.34                          |
| 12                        | 6   | 2    | 5.2                   | 7.0     | 23.3                | 1.02                          |
| 12                        | 6   | 10   | 4.4                   | 7.5     | 29.2                | 2.48                          |
| 12                        | 6   | 20   | 4.4                   | 8.3     | 28.4                | 1.25                          |
| Control                   |     |      | 10.1                  | 20.9    | 30.5                | 0.51                          |

Shrinkages were determined as in Example 2, and stiffness was determined by the Peirce heart loop method. Tensile strength was found by a Scott inclined plane tester on strips 38 ends wide with one inch between clamps.

It will be seen from the above example that all of the treated fabrics show better shrinkage and stiffness characteristics than the untreated fabric.

#### Example 4

In the following example, the time of application of the solution to a cotton marquisette fabric of the type described in Example 3 was varied from 1 second to 24 hours. In each case, following contact of the solution with the fabric, the latter was dried under tension, after which the fabric was washed and dried. The solution used was the same for all samples and contained 12% caustic, 6% zinc oxide and 10% urea. In some cases the washing procedure and the final drying step were varied.

under tension, given an acid wash followed by a water rinse, and dried on a frame. No difficulty was experienced in framing these samples to their original width. The results are as follows:

| 5       | Sample | Time of Application of Solution | Time Fabric Allowed to Remain Moist | Shrinkage |          | Tensile Strength |
|---------|--------|---------------------------------|-------------------------------------|-----------|----------|------------------|
|         |        |                                 |                                     | Warp      | Filling  |                  |
| 10      |        | Seconds                         | Minutes                             | Per cent  | Per cent | Pounds           |
| 1       |        | 1                               | 10                                  | 3.9       | 5.5      | 24.4             |
| 2       |        | 1                               | 30                                  | 4.7       | 4.5      | 24.8             |
| 3       |        | 1                               | 60                                  | 4.8       | 5.8      | 23.3             |
| Control |        | 1                               |                                     | 18.5      | 21.3     | 21.3             |

15 <sup>1</sup> Treated with water, not solution.

#### Example 6

Samples of mercerized, kier boiled and bleached 20 80 x 80 cotton print cloth were padded in the unstretched condition with the solution of Example 4 for various times. The samples were then dried on a frame, taken off the frame and neutralized with acid, rinsed, and finally dried on a frame. The results are as follows:

| 25      | Sample | Time of Application of Solution | Shrinkage |          | Tensile Strength | Stiffness Coefficient |
|---------|--------|---------------------------------|-----------|----------|------------------|-----------------------|
|         |        |                                 | Warp      | Filling  |                  |                       |
| 30      |        | Seconds                         | Per cent  | Per cent | Pounds           |                       |
| 1       |        | 1                               | 4.3       | 4.6      | 60.9             | 1.40                  |
| 2       |        | 10                              | 3.7       | 3.4      | 64.4             | 3.88                  |
| Control |        | 10                              | 6.1       | 6.9      | 56.1             | 0.58                  |

35 <sup>1</sup> Treated with water, not solution.

In a modification of the foregoing solution treating process the cloth is subjected to the action of a chemical degradation agent and then 40 treated with the solution as described. The object of the degradation step is to render the cloth more susceptible to the action of the solution, but care must be exercised to limit the amount of degradation. To this end the strength 45 of the agent and the time and temperature of its application are carefully controlled.

| Solution Application |                 |                             | Washing                     | Drying under Tension | Shrinkage |          | Tensile Strength | Stiffness Coefficient |
|----------------------|-----------------|-----------------------------|-----------------------------|----------------------|-----------|----------|------------------|-----------------------|
| Sample               | Time            | Tensioning during Treatment |                             |                      | Warp      | Filling  |                  |                       |
| 1                    | 24 hrs.         | Yes                         | Acid wash plus water rinse. | Yes                  | Per cent  | Per cent | Pounds           |                       |
|                      |                 |                             |                             |                      | 3.8       | 5.4      | 28.8             | 1.50                  |
| 2                    | do              | No                          | Like 1                      | do                   | 5.3       | 7.8      | 36.3             | 1.80                  |
| 3                    | 1 sec.          | do                          | do                          | do                   | 4.0       | 8.0      | 34.0             | 0.91                  |
| 4                    | do              | do <sup>2</sup>             | do                          | do                   | 4.3       | 7.3      | 32.5             | 1.08                  |
| 5                    | 1 min.          | Yes                         | do                          | do                   | 4.2       | 6.2      | 32.6             | 2.27                  |
| 6                    | do              | No                          | do                          | do                   | 3.3       | 5.1      | 38.3             | 1.24                  |
| 7                    | do              | Yes                         | do                          | No-Dried Flat        | 1.6       | 2.8      | 28.0             | 1.59                  |
| 8                    | do              | do                          | Hot Water                   | Yes                  | 3.2       | 8.9      | 28.8             | 0.72                  |
| Control              | do <sup>1</sup> | do                          | Like 1                      | do                   | 10.1      | 20.9     | 30.5             | 0.51                  |

<sup>1</sup> Treated with water, not solution.

<sup>2</sup> But kept under tension for 24 hrs. while moist with solution.

#### Example 5

In the following tests, cotton marquisette, similar to that of Examples 3 and 4, after the padding of solution (the same solution as in the preceding example) on the same in unstretched condition, was allowed to remain wet with the solution for various periods of time and while still unstretched. Thereafter the fabric was dried 70 75

The degradation agent to be employed may be a bleaching compound such as the alkali and alkaline earth metal hypochlorites, of which group sodium hypochlorite is a preferred material, hypochlorous acid, and sodium chlorite. Hydrogen peroxide, or ammonium persulphate, which are conventional bleaching agents, are useful, as is a combination of sodium peroxide, or

other alkali metal and alkaline earth metal peroxides, and sulfuric acid. Sodium peroxide may be employed with other acids, such as boric acid, and may be used alone, as may sodium perborate which breaks down to yield the peroxide. Other agents include oxidizing materials such as permanganate and bichromate alone or in conjunction with sulfuric, oxalic, or other acids.

In the case of the chlorine-containing agents, the strength of the solution should not be below 0.1% available chlorine. Stronger solutions may be used, going up to 5 or 10%, or higher. Whatever concentration is employed, it must be correlated with the treating time and the temperature. Thus, using sodium hypochlorite, it has been found that the hypochlorite has a two-fold effect on the fabric: it lowers the shrinkage, and it decreases the tensile strength. Example 7 shows the effect of hypochlorite concentration and treating time upon the tensile strength of a marquisette fabric at 25° C. Preferred treating temperatures range from room temperature to about 80° F., although higher or lower temperatures may be used. Treating periods may range from 20 to 60 minutes. In the case of hypochlorite, for example, illustrative operating conditions would be as follows (see Example 7): temperature, 25° C.; treating time, 30 minutes; available chlorine concentration, 0.1 to 2.3%.

In applying the hypochlorite degradation agent to the cloth, the latter is maintained in an unstretched condition and may be impregnated with a solution of the agent or immersed therein. When immersion is employed, the cloth may be agitated in the solution. The cloth may then be washed, and thereafter it is carefully dried and framed.

The next step in the treatment of the cloth according to this modification is the application of the caustic zincate-urea solution, which, to a notable degree, serves to stabilize the cloth against shrinkage, as well as to clarify it. In applying this solution, the conditions to be employed are substantially the same as described above in connection with the single step process. The following example illustrates the variation in tensile strength with hypochlorite treating conditions obtainable by the two stage process:

*Example 7*

A series of runs were made in which marquisette cloth (unstretched) in 3.5 gm. pieces were tumbled at 25° C. for 30 minutes in a number of sodium hypochlorite solutions ranging from below 0.1% available chlorine to about 5.4%. Another group of samples were subjected to identical treatment except that a treating time of 60 minutes was used. The goods were then washed with cold water, rinsed with 1% hydro-sulfite solution (antichlor) and then water again. Each sample was dried at 220° F. for about two minutes, framed, and saturated with the caustic zincate-urea solution (4.5% zinc oxide, 10% caustic, and 10% urea). Each was then placed in a current of hot air until the material felt just dry, rinsed in water at about 100° F., washed with cold 5% acetic acid, and finally with water until neutral. The samples were then dried at about 220° F. and removed from the stretching frame. Tensile strengths of the samples were

8  
determined according to the procedure above indicated. Following are the results:

| Available Chlorine, Per Cent by weight | Overall Loss in Tensile Strength, Per Cent Hypochlorite Treating Time |         |
|----------------------------------------|-----------------------------------------------------------------------|---------|
|                                        | 30 Min.                                                               | 60 Min. |
| 0.1                                    | 11.3                                                                  | 12      |
| 0.5                                    | 14.2                                                                  | 16.7    |
| 1.0                                    | 17.8                                                                  | 21.8    |
| 2.0                                    | 23.8                                                                  | 29.8    |
| 2.3                                    | 25                                                                    | 32      |
| 3.0                                    | 28.8                                                                  | 36      |
| 4.0                                    | 32.7                                                                  | 41.5    |
| 5.0                                    | 36.4                                                                  | 47      |

These figures are based upon the tensile strength as measured at the conclusion of the overall process, and therefore include any change due to the caustic zincate-urea solution.

The concentrations of the other degradation agents will, of course, be different from those obtaining in the case of hypochlorite, and will also vary among themselves, depending upon the agent and the particular treating conditions employed. Therefore no general numerical range covering them collectively can be given in terms of concentration, but for all of them the concentration must be such as not to effect an excessive overall loss in tensile strength. Such concentrations, as indicated, will vary with the temperature and the time of treatment, lower concentrations being suitable with longer times and higher temperatures, and vice versa. Conditions suitable for use with these degradation agents may be found in Example 9 below.

In a second modification of the solution treating process, the cloth is given a chemical degradation, then treated with the solution, and finally treated with a special stiffening liquor. By this process a greatly increased stiffness is imparted to the cloth, in addition to the stabilization and clarification effects which result from the degradation and solution treating steps. The overall result of this modified or three stage process is more than merely the added effect of the stiffening liquor, for it has been found, as shown below, that the loss in tensile strength incurred by the first two stages of the process is reduced in the third stage, i. e., the fabric gains strength by treatment with the stiffening liquor. Moreover, as pointed out in Example 2, the step of drying the solution on the cloth resulted in better stiffness. In the three stage process, the use of the stiffening liquor affords the advantage of a greater stiffness effect and with increased stiffness there are also obtained improved clarification and shrinkage or dimensional stabilization effects.

In practicing the three stage process, the cloth is first subjected to the action of the degradation agent and then to the solution treating operation as described heretofore. It is then ready for the stiffening liquor. The latter may have a composition as follows: about 20 to 35% by weight of an alkali metal hydroxide selected from the class consisting of sodium hydroxide and potassium hydroxide; about 2 to 6% by weight of zinc oxide; and about 8 to 12% by weight of urea. A preferred range for the sodium hydroxide is from about 20 to about 25%. For potassium, a range of from about 28 to about 35% is preferred. A preferred composition is: sodium hydroxide 22%, zinc oxide 4% and urea 10%.

Treating times with the stiffening liquor may vary from about ten seconds to about two minutes. Treating temperatures above and below room temperature may be used, although room temperature is preferred. The liquor is applied

ent degradation agents upon the cloth with respect to tensile strength, stiffness, and shrinkage. Samples of cotton marquisette that had been conventionally kier boiled and which had the following characteristics were used:

| Weight/sq.<br>yds., ounces,<br>Max. | Thread Count<br>per inch |         | Breaking Strength<br>1 x 1 x 3 Grab,<br>Pounds, Min. |         | Meshes per<br>sq. in. | Size of<br>Hole,<br>Max. |
|-------------------------------------|--------------------------|---------|------------------------------------------------------|---------|-----------------------|--------------------------|
|                                     | Warp                     | Filling | Warp                                                 | Filling |                       |                          |
|                                     |                          |         | 28                                                   | 20      |                       |                          |
| 1.8                                 | 50-52                    | 50-52   | 28                                                   | 20      | 625-676               | 0.03 x 0.0325            |

to the fabric in any desired manner while the latter is under tension, or not, as desired.

The following example illustrates the strengthening effect of the stiffening solution:

*Example 8*

Marquisette that had been kier boiled was cut into a number of 14" x 20" pieces and these were subjected to degradation treatments by tumbling for 60 minutes at 25° C. in sodium hypochlorite solutions ranging from 0.1 to 5.4% available chlorine. After the usual rinsing, the samples were dried at 220° F. for about two minutes. They were then framed to original width and treated for one minute with the caustic zincate-urea solution (10% caustic, 4.5% zinc oxide, 10% urea) at 25° C. Thereafter they were rinsed

Samples of this marquisette were treated with different degradation agents at normal treating conditions for each agent. Then the loss in tensile strength of each sample was measured. Following this, each sample was subjected to the solution treating step comprising a 1- to 2-minute treatment at 25° C. with a solution containing 10% caustic, 4.5% zinc oxide, and 10% urea. The solution was washed from the samples before drying the same. The usual scouring, washing, drying and framing conditions were observed. Thereafter, each sample was treated with a stiffening liquor containing 22% caustic, 4% zinc oxide, and 10% urea, for one to two minutes at 25° C., again observing the usual auxiliary operations. Results of these treatments are as follows:

| Sample                                                                               | Loss in Tensile<br>Strength |                             | Stiffness,<br>Bending<br>Force in<br>Gms. | Shrinkage,<br>Per Cent |         |
|--------------------------------------------------------------------------------------|-----------------------------|-----------------------------|-------------------------------------------|------------------------|---------|
|                                                                                      | After<br>Degrad.            | After<br>Overall<br>Process |                                           | Warp                   | Filling |
| Original Cloth                                                                       |                             |                             | 0.05                                      | 12                     | 20      |
| Original Cloth, starched                                                             |                             |                             |                                           | 10.1                   | 18.1    |
| Degraded Cloth (Degrading agent and conditions):                                     |                             |                             |                                           |                        |         |
| NaOCl (1.25% available Cl <sub>2</sub> ) 60<br>min. at 25° C.                        | 20                          | 16                          | .27                                       | 3.5                    | 5.2     |
| KMnO <sub>4</sub> (1%) in H <sub>2</sub> SO <sub>4</sub> (2%) 1 min.<br>at 25° C.    | 26                          | 28.5                        | .38                                       | 5.0                    | 2.6     |
| KMnO <sub>4</sub> (1%) in Na <sub>2</sub> CO <sub>3</sub> (2%) 0.5<br>min. at 25° C. | 25.5                        | 32                          | .38                                       | 4.6                    | 2.8     |
| H <sub>2</sub> SO <sub>4</sub> (35%) 5 min. at 25° C.                                | 19                          | 20                          | .28                                       | 3.8                    | 4.7     |

Figures enclosed in parentheses refer to concentrations.

with water, 5% acetic acid, and water again, and dried at 220° F. for two minutes. They were then framed, given a one-minute treatment with the stiffening liquor (22% caustic, 4% zinc oxide, 10% urea) at 25° C., rinsed and dried as before. Tensile strength data, measured as described, are as follows:

| Available<br>Chlorine,<br>Per Cent | Loss in Tensile Strength,<br>Per Cent |                             |
|------------------------------------|---------------------------------------|-----------------------------|
|                                    | After<br>Degradation<br>Stage         | After<br>Overall<br>Process |
| 0.1                                | 4.0                                   | 0.2                         |
| 0.5                                | 11.3                                  | 6.8                         |
| 1.0                                | 16.0                                  | 11.6                        |
| 1.5                                | 18.9                                  | 14.5                        |
| 2.0                                | 21.0                                  | 16.5                        |
| 2.5                                | 22.4                                  | 17.8                        |
| 3.0                                | 23.7                                  | 18.5                        |
| 3.5                                | 24.8                                  | 18.9                        |
| 4.0                                | 25.8                                  | 19.3                        |
| 4.5                                | 26.6                                  | 19.6                        |
| 5.4                                | 27.5                                  | 19.6                        |

*Example 9*

In this example is shown the effect of differ-

ent degradation agents upon the cloth with respect to tensile strength, stiffness, and shrinkage. It will be observed that in the case of the hypochlorite, subsequent treatment with the solution and the stiffening liquor served to reduce the loss in tensile strength. Tensile strength, stiffness, and shrinkage were determined according to methods heretofore described. The data on stiffness and shrinkage were obtained at the conclusion of the overall process.

*Example 10*

In order to compare the results obtainable by the present process with those of a commercial sulfuric acid process, a sample of cotton marquisette was kier boiled and partially mercerized according to customary plant treatment and then subjected to the following treatment: (a) degradation with sodium hypochlorite, 1.25% available chlorine, for 60 minutes at 40° F.; (b) a solution treatment for one minute at 40° F., the solution being the same as in Example 8; (c) treatment with a stiffening liquor for one minute at 40° F., the liquor being the same as in Example 8. This sample and a cotton marquisette of the same construction but finished according to the commercial sulfuric acid method were then tested, the shrinkage and stiffness data on

## 11

the former being reported as at the end of the overall process.

|                                                          | Present Process | Commercial Acid Process |
|----------------------------------------------------------|-----------------|-------------------------|
| Tensile strength of warp threads per inch of width, lbs. | 1 27.2          | 2 28.5                  |
| Shrinkage, Per Cent:                                     |                 |                         |
| Warp                                                     | 2.9             | 4.3                     |
| Filling                                                  | 3.3             | 6.9                     |
| Stiffness, gms.                                          | 0.63            | 0.58                    |

<sup>1</sup> After plant treatment.

<sup>2</sup> Finished cloth.

As will be seen, the present process yielded a cloth of superior shrinkage quality, while the stiffness results are of the same order as commercial samples which are noted for their stiffness qualities.

Besides the foregoing processes involving one, two, and three stages, useful effects may be attained by various alternative processes in which the sequence of operations may be as follows: (1) degrade—apply stiffening liquor—apply solution—apply stiffening liquor, or (2) degrade—apply solution—apply stiffening liquor—apply solution. In still other alternative methods, the degradation step of the last-mentioned sequences may be omitted, thus offering advantages in time and material saved, although the results, while satisfactory for some purposes, may not be as good as those to be obtained in the one, two and three stage processes described above in detail.

## Example 11

Samples of the same leno weave cotton marquisette used in Example 3 were held under moderate tension on a frame and treated at room temperature with various solutions in which sodium hydroxide and sodium zincate had been replaced by potassium hydroxide and potassium zincate. The treatment of the samples was carried out in the manner described in Example 3. Amounts of potassium hydroxide corresponding to the minimum, preferred and maximum concentrations of sodium hydroxide were used. Samples treated with the minimum, preferred and maximum compositions of sodium hydroxide, zinc oxide and urea were included for comparison. The results are as follows:

| KOH  | Solution Composition, Per Cent |     |      |      | Shrinkage |      | Tensile Strength Warp<br>Pounds | Stiffness Coefficient |
|------|--------------------------------|-----|------|------|-----------|------|---------------------------------|-----------------------|
|      | NaOH                           | ZnO | Urea | Warp | Filling   |      |                                 |                       |
|      |                                |     |      |      |           |      |                                 |                       |
| 6    | —                              | 2   | 2    | 9.0  | 12.0      | 22.2 | .405                            |                       |
| 8.4  | 6                              | 2   | 2    | 7.5  | 10.4      | 24.5 | .96                             |                       |
| 16.8 | 6                              | 6   | 10   | 7.3  | 9.3       | 25.4 | .59                             |                       |
| 28   | 12                             | 6   | 10   | 4.0  | 5.3       | 28.9 | .72                             |                       |
| —    | —                              | 10  | 20   | 4.0  | 7.8       | 29.4 | 3.75                            |                       |
| —    | 20                             | 10  | 20   | 5.5  | 8.3       | 30.9 | 1.94                            |                       |
| —    | 28                             | 10  | 20   | 5.1  | 6.7       | 24.3 | 1.032                           |                       |

In conclusion, it is to be noted that in place of urea per se or the urea forming compounds as described, other compounds may be employed as one of the components in the present treating solution as, for examples, the alkali metal thiocyanates; sodium thiocyanate, potassium thiocyanate or ammonium thiocyanate, and the poly-aminies; ethylene diamine or hexamethylene-tetramine.

This application is a continuation in part of copending application Serial Number 616,451, filed September 14, 1945 now abandoned.

## 12

What is claimed is:

1. Process of modifying cotton fabric which includes the steps of treating the same with an aqueous solution comprising from about 2 to about 20% by weight of urea, an alkali metal zincate selected from the class consisting of sodium zincate and potassium zincate in an amount equivalent to from about 2 to about 10% by weight of zinc oxide, from about 6 to about 28% by weight of alkali metal hydroxide selected from the class consisting of sodium hydroxide and potassium hydroxide, and the balance water, for a time ranging from about 1 second to about 24 hours, drying the treated fabric while under tension, neutralizing the same and thereafter rinsing the fabric.

2. Process of modifying cotton fabric which includes the steps of treating the same with an aqueous solution comprising from about 2 to about 20% by weight of urea, an alkali metal zincate selected from the class consisting of sodium zincate and potassium zincate in an amount equivalent to from about 2 to about 10% by weight of zinc oxide, from about 6 to about 28% by weight of alkali metal hydroxide selected from the class consisting of sodium hydroxide and potassium hydroxide, and the balance water, for a time ranging from about 1 second to about 24 hours, drying the treated fabric while under tension and neutralizing the same.

3. Process of modifying cotton fabric which includes the steps of treating the same with an aqueous solution comprising from about 2 to about 20% by weight of urea, an alkali metal zincate selected from the class consisting of sodium zincate and potassium zincate in an amount equivalent to from about 2 to about 10% by weight of zinc oxide, from about 6 to about 28% by weight of alkali metal hydroxide selected from the class consisting of sodium hydroxide and potassium hydroxide, and the balance water, for a time ranging from about 1 second to about 24 hours, drying the treated fabric while under tension and thereafter washing the solution therefrom.

4. Process of modifying cotton fabric which includes the steps of treating the same with an aqueous solution comprising from about 2 to about 20% by weight of urea, an alkali metal zincate selected from the class consisting of sodium zincate and potassium zincate in an amount equivalent to from about 2 to about 10% by weight of zinc oxide, from about 6 to about 28% by weight of alkali metal hydroxide selected from the class consisting of sodium hydroxide and potassium hydroxide, and the balance water, for a time ranging from about 1 second to about 24 hours, drying the treated fabric while under tension and thereafter neutralizing and rinsing the same.

5. Process of modifying cotton fabric which includes the steps of treating the same with an aqueous solution comprising from about 2 to about 20% by weight of urea, an alkali metal zincate selected from the class consisting of sodium zincate and potassium zincate in an amount equivalent to from about 2 to about 10% by weight of zinc oxide, from about 6 to about 28% by weight of alkali metal hydroxide selected from the class consisting of sodium hydroxide and potassium hydroxide, and the balance water, for a time ranging from about 1 second to about 24 hours, drying the treated fabric and thereafter neutralizing the same.

6. Process of modifying cotton fabric which includes the steps of treating the same with an

aqueous solution comprising from about 2 to about 20% by weight of urea, an alkali metal zincate selected from the class consisting of sodium zincate and potassium zincate in an amount equivalent to from about 2 to about 10% by weight of zinc oxide, from about 6 to about 28% by weight of alkali metal hydroxide selected from the class consisting of sodium hydroxide and potassium hydroxide, and the balance water, for a time ranging from about 1 second to about 24 hours, drying the treated fabric and then washing the solution therefrom.

7. Process of modifying cotton fabric which includes the steps of treating the same with an aqueous solution comprising from about 2 to about 20% by weight of urea, an alkali metal zincate selected from the class consisting of sodium zincate and potassium zincate in an amount equivalent to from about 2 to about 10% by weight of zinc oxide, from about 6 to about 28% by weight of alkali metal hydroxide selected from the class consisting of sodium hydroxide and potassium hydroxide, and the balance water, for a time ranging from about 1 second to about 24 hours, neutralizing the treated fabric and rinsing the same

8. Process of modifying cotton fabric which includes the steps of treating the same with an aqueous solution comprising from about 2 to about 20% by weight of urea, an alkali metal zincate selected from the class consisting of sodium zincate and potassium zincate in an amount equivalent to from about 2 to about 10% by weight of zinc oxide, from about 6 to about 28% by weight of alkali metal hydroxide selected from the class consisting of sodium hydroxide and potassium hydroxide, and the balance water, for a time ranging from about 1 second to about 24 hours, and thereafter neutralizing the treated fabric.

9. Process of modifying cotton fabric which includes the steps of treating the same with an aqueous solution comprising from about 2 to about 20% by weight of urea, an alkali metal zincate selected from the class consisting of sodium zincate and potassium zincate in an amount equivalent to from about 2 to about 10% by weight of zinc oxide, from about 6 to about 28% by weight of alkali metal hydroxide selected from the class consisting of sodium hydroxide and potassium hydroxide, and the balance water, for a time ranging from about 1 second to about 24 hours, and then washing the solution from the treated fabric.

10. Method of modifying cotton fabric which includes the steps of treating the same with an aqueous solution comprising from about 2 to about 20% by weight of urea, sodium zincate equivalent to from about 2 to about 10% by weight of zinc oxide, from about 6 to about 20% by weight of sodium hydroxide, and the balance water, for a time ranging from about 1 second to about 24 hours and subsequently removing the solution from the treated fabric.

11. Method of modifying cotton fabric which includes the steps of treating the same with an aqueous solution comprising from about 2 to about 20% by weight of urea, potassium zincate equivalent to from about 2 to about 10% by weight of zinc oxide, from about 8 to about 28% by weight of potassium hydroxide, and the balance water, for a time ranging from about 1 second to about 24 hours and subsequently removing the solution from the treated fabric.

12. Method of modifying cotton fabric which includes the steps of treating the same with an aqueous solution comprising from about 2 to about 20% by weight of urea, sodium zincate equiva-

lent to from about 2 to about 10% by weight of zinc oxide, from about 6 to about 28% by weight of sodium hydroxide, and the balance water, for a time ranging from about 1 second to about 24 hours, and subsequently removing the solution from the treated fabric.

13. Method of modifying cotton fabric which includes the steps of treating the same with an aqueous solution comprising from about 2 to about 20% by weight of urea, potassium zincate equivalent to from about 2 to about 10% by weight of zinc oxide, from about 6 to about 28% by weight of potassium hydroxide, and the balance water, for a time ranging from about 1 second to about 24 hours and subsequently removing the solution from the treated fabric.
- 14.
- 15.

14. Process of modifying cotton fabric which includes the steps of treating the same with an aqueous solution comprising from about 2 to about 20% by weight of urea, an alkali metal zincate selected from the class consisting of sodium zincate and potassium zincate in an amount equivalent to from about 2 to about 10% by weight of zinc oxide, from about 6 to about 28% by weight of alkali metal hydroxide selected from the class consisting of sodium hydroxide and potassium hydroxide, and the balance water, for a time ranging from about 1 second to about 24 hours, and subsequently removing the solution from the treated fabric.

15. Process of modifying the characteristics of cotton fabric which includes the steps of subjecting said fabric in an unstretched condition to the action of an oxidizing agent to obtain a partial degradation of the fabric, and thereafter treating the partially degraded fabric with an aqueous solution comprising from about 2 to about 35% by weight of urea, an alkali metal zincate selected from the class consisting of sodium zincate and potassium zincate in an amount equivalent to from about 2 to about 10% by weight of zinc oxide, from about 6 to about 28% by weight of alkali metal hydroxide selected from the class 40 consisting of sodium hydroxide and potassium hydroxide, and the balance water, for a time ranging from about 1 second to about 24 hours, and subsequently removing the solution from the 45 fabric.

16. Process of modifying the characteristics of cotton fabric which includes the steps of subjecting said fabric in an unstretched condition to the action of an oxidizing agent to obtain a partial degradation of the fabric, and thereafter treating the partially degraded fabric with an aqueous solution comprising from about 2 to about 20% by weight of urea, sodium zincate in an amount equivalent to from about 2 to about 10% by weight of zinc oxide, from about 6 to about 20% by weight of sodium hydroxide, and the balance water, for a time ranging from about 1 second to about 24 hours, and subsequently removing the solution from the fabric.

17. Process of modifying cotton fabric which includes the steps of subjecting said fabric in an unstretched condition to the action of an oxidizing agent to obtain a partial degradation of the fabric, treating said partially degraded fabric with an aqueous solution comprising from about 2 to about 20% by weight of urea, an alkali metal zincate selected from the class consisting of sodium zincate and potassium zincate equivalent to from about 2 to about 10% by weight of zinc oxide, and from about 6 to about 28% by weight of alkali metal hydroxide selected from the class consisting of sodium hydroxide and potassium

15

hydroxide, for a time ranging from about 1 second to about 24 hours, removing the solution from the fabric and thereafter subjecting the partially degraded and treated fabric to the action of an aqueous stiffening liquor comprising from about 8 to about 12% by weight of urea, an alkali metal zincate selected from the class consisting of sodium zincate and potassium zincate in an amount equivalent to from about 2 to about 6% by weight of zinc oxide and from about 20 to about 35% by weight of alkali metal hydroxide selected from the class consisting of sodium hydroxide and potassium hydroxide, and removing the stiffening liquor from the fabric.

18. Process of modifying cotton fabric which includes the steps of subjecting the fabric in an unstretched condition to the action of an oxidizing agent to obtain a partial degradation of the fabric, treating said partially degraded fabric with an aqueous solution comprising from about 2 to about 20% by weight of urea, sodium zincate equivalent to from about 2 to about 10% by weight of zinc oxide, and from about 6 to about 20% by weight of sodium hydroxide, for a time ranging from about 1 second to about 24 hours, removing the solution from the fabric, and thereafter subjecting the partially degraded and treated fabric to the action of an aqueous stiffening liquor comprising from about 8 to about 12% by weight of urea, sodium zincate in an amount equivalent to from about 2 to about 6% by weight of zinc oxide, and from about 20 to about 25% by weight of sodium hydroxide, and removing the stiffening liquor from the fabric.

19. Process of modifying cotton fabric which includes the steps of treating the same with an aqueous solution comprising about 10 per cent by weight of urea, sodium zincate in an amount equivalent to about 6 per cent by weight of zinc oxide, about 12 per cent by weight of sodium

hydroxide and the balance water, for a time of about one minute, drying the treated fabric under tension, and subsequently neutralizing, rinsing, and drying the fabric.

5 20. Process of modifying cotton fabric which includes the steps of treating the same with an aqueous solution comprising about 10 per cent by weight of urea, sodium zincate in an amount equivalent to about 6 per cent by weight of zinc oxide, about 12 per cent by weight of sodium hydroxide and the balance water, for a time of about one minute, drying the treated fabric under tension, subsequently neutralizing and rinsing the fabric in an unstretched condition, and finally drying the fabric under tension.

15 CHARLES L. MANTELL.  
OSCAR K. HEIM.

## REFERENCES CITED

20 The following references are of record in the file of this patent:

## UNITED STATES PATENTS

| Number    | Name      | Date           |
|-----------|-----------|----------------|
| 1,630,365 | Weber     | May 31, 1927   |
| 1,661,879 | DeGoncz   | Mar. 6, 1928   |
| 2,129,708 | Schreiber | Sept. 13, 1938 |
| 2,142,043 | Boyd      | Dec. 27, 1938  |
| 2,203,375 | Weiss     | June 4, 1940   |

## FOREIGN PATENTS

| Number  | Country       | Date          |
|---------|---------------|---------------|
| 20,314  | Great Britain | 1889          |
| 266,466 | Great Britain | Feb. 24, 1927 |
| 516,843 | Great Britain | Jan. 12, 1940 |

## OTHER REFERENCES

Katz et al., Rayon Text. Mo., Dec. 1940, pages 40 54, 55.